

## UNITED STATES PATENT OFFICE

2,260,455

## WIRED DRAWING

Charles Richard Horwedel, Lakewood, Ohio, assignor to The American Steel and Wire Company of New Jersey, a corporation of New Jersey

No Drawing. Application May 21, 1940,  
Serial No. 336,441

5 Claims. (Cl. 205—21)

This invention is a method of drawing wire by means of a wire wet-drawing machine or its equivalent.

Such a machine includes a box containing two rotatively powered blocks each providing a plurality of drum surfaces that progressively increase in diameter and a series of dies, the arrangement being such that the wire is continuously drawn successively through the dies which successively decrease in orifice diameter, the wire going back and forth from block to block by way of wrapping around their various drum surfaces, the diameter increases of the latter taking care of the elongation of the wire. Drawing speeds are usually high and the machine includes a system for continuously bathing the wire, dies and drum surfaces with a liquid coolant, the box of the machine preventing coolant loss. The coolant is water which may sometimes contain soap in solution to aid in reducing die wear.

When stainless steel wire is drawn by such a machine the dies of the machine are drilled diamonds because the metal is hard and the diameter tolerance ranges of such wire are generally narrow. Sometimes other die material may be used but in all cases it is expensive. Hence it is desirable to prolong the die life as much as possible. The present practice of using soap in the coolant leaves much to be desired in this direction, the invention now to be described having proven a great improvement in actual practice, it being now in commercial use in connection with drawing stainless steel wire by wire wet-drawing machines using diamond dies.

In accordance with this invention, stainless steel wire ready for wet-drawing is run through molten wax having a melting temperature not less than 40 degrees centigrade. The arrangement used consists of a pan in front of the wet-drawing machine and heated by a Bunsen burner as required to keep the wax liquid, the wire traveling a sufficient distance through the atmosphere before entering the machine to assure its solidifying before encountering the first of the dies. Beeswax is used successfully, its melting temperature being from 62 degrees to 70 degrees centigrade. Also applicable are Chinese wax with a melting temperature of from 80 degrees to 81 degrees centigrade, paraffin with a melting temperature of from 47 degrees to 52 degrees centigrade, bayberry wax melting at from 40 degrees to 48 degrees centigrade, and carnauba wax with a melting temperature of from 83 degrees to 91 degrees centigrade. The choice is determined by economics, the wax with the highest melting tem-

perature that can be obtained at a proper price being the one to use.

The wire now coated with solid wax then encounters the first die of the machine and there it melts due to the heat and pressure incidental to the draw. Thus a very effective lubrication action is obtained, the transition of solid to liquid wax being in accordance with the transition of no pressure to full drawing pressure as exerted by the die, the wax having decreasing viscosity to continuously meet the increasing pressure, all in accordance with good lubricating engineering. This result cannot be had by using soap in the coolant, it being eliminated in the practice of this invention, if desired, and plain water used instead.

Immediately upon leaving this first die, the wax is solidified by the coolant of the machine so as to be ready to repeat its above described result at the next die. As long as the wire is being worked by the machine, it is being successively melted as the wire draws through the dies and successively hardened as it goes from die to die. This follows when the coolant is maintained at its normal temperature in most circumstances, though in hot weather it may be necessary to provide for lowering the coolant temperature beyond the capacity of the normal machine. This merely means that the coolant must be passed through a cooler of prior art design, it being understood that the usual machine provides for circulating the coolant continuously.

Since the machine provides for bathing the wire leaving the last of the series of its dies, the wax coating is retained on the wire leaving the machine. This coating is of advantage in many instances to the ultimate user of the wire and should not be removed in most cases. Thus it prevents scratching of the wire when it is worked by helical spring coiling machines and the like.

Summarizing the invention, it may be said to be, specifically speaking, a method of continuously drawing stainless steel wire through a series of spaced diamond or other expensive dies, the method being characterized by coating the wire with a solid wax, drawing the wire successively through the dies, the wax melting as the wire draws through each die, and bathing the wire with a fluid coolant as it passes from die to die so as to solidify the wax melted in preceding dies and keep it on the wire so it can function as an initially solid lubricant in succeeding dies, the wax having a melting temperature of not less than 40 degrees centigrade and being bathed by the coolant upon leaving the

last die so the wire retains a wax coating to facilitate its further processing or manipulation.

This is the invention as it is now commercially worked but its principles may prove applicable to the solving of other troubles than that of rapid wear of diamond dies by stainless steel wire in the continuous wet-drawing process.

I claim:

1. A method of drawing wire in a continuous wire wet-drawing machine, the method being characterized by coating the wire with wax prior to its entering the dies of the machine, the wax having a melting temperature resulting in its being successively melted as it draws through the dies of the machine and successively hardened by the liquid used by the machine to bathe the wire and dies during the travel of the wire from die to die.

2. A method of reducing the wear on the dies of a continuous wire wet-drawing machine working hard metal wire such as stainless steel wire, the method being characterized by coating such wire with wax prior to its entering the dies of the machine, the wax having a melting temperature of not less than 40 degrees centigrade.

3. A method of continuously drawing stainless steel wire through a series of spaced diamond or other expensive dies, the method being characterized by coating the wire with a solid wax, drawing the wire successively through the dies, the wax melting as the wire draws through each die, and bathing the wire with a fluid coolant as

it passes from die to die so as to solidify the wax melted in preceding dies and keep it on the wire so it can function as an initially solid lubricant in succeeding dies.

4. A method of continuously drawing stainless steel wire through a series of spaced diamond or other expensive dies, the method being characterized by coating the wire with a solid wax, drawing the wire successively through the dies, the wax melting as the wire draws through each die, and bathing the wire with a fluid coolant as it passes from die to die so as to solidify the wax melted in preceding dies and keep it on the wire so it can function as an initially solid lubricant in succeeding dies, the wax having a melting temperature of not less than 40 degrees centigrade.

5. A method of continuously drawing stainless steel wire through a series of spaced diamond or other expensive dies, the method being characterized by coating the wire with a solid wax, drawing the wire successively through the dies, the wax melting as the wire draws through each die, and bathing the wire with a fluid coolant as it passes from die to die so as to solidify the wax melted in preceding dies and keep it on the wire so it can function as an initially solid lubricant in succeeding dies, the wax having a melting temperature of not less than 40 degrees centigrade and being bathed by the coolant upon leaving the last die so the wire retains a wax coating to facilitate its further processing or manipulation.

CHARLES RICHARD HORWEDEL.